

## UNITED STATES PATENT OFFICE

2,363,394

## HEAT TREATMENT OF MAGNESIUM ALLOYS

Robert S. Bush, Midland, Mich., assignor to The Dow Chemical Company, Midland, Mich., a corporation of Michigan

No Drawing. Application December 23, 1943,  
Serial No. 515,419

7 Claims. (Cl. 148—21.3)

This invention relates to the heat-treatment of magnesium-base alloys. It particularly concerns a preliminary sequence for minimizing germination during solution-heat-treatment of magnesium-base alloy castings.

During the heat-treatment of metals, there is sometimes observed the phenomenon of germination, or sporadic uncontrolled grain growth. (See, for example, the discussion in "The Science of Metals," p. 133 ff., Jeffries and Archer, McGraw-Hill, New York, 1924.) Thus, after prolonged solution-heat-treatment of certain magnesium-base alloy castings, local areas of the metal may exhibit, instead of the usual large number of small grains, one or a few relatively enormous grains having a diameter of a tenth of an inch or more; single grains more than half an inch in size are occasionally seen. Inasmuch as the occurrence of such macro-crystalline areas may so weaken the metal as to render it unfit for service, the avoidance of germination during heat-treatment of magnesium alloys is of great practical importance.

According to the present invention, uncontrolled crystal growth during heat-treatment of heat-treatable magnesium-base alloys characterized by a tendency toward germination may be largely prevented by a pre-treatment which comprises heating the metal at a solution-heat-treating temperature for a time sufficient to effect partial solution of any major second phase present but insufficient to cause appreciable germination, and then cooling the metal and subjecting it to an aging temperature for a time sufficient to effect substantial precipitation of a major second phase. This pre-treatment, involving partial solution and reprecipitation of a major second phase present in the alloy, appears to alter the ultimate structure of the metal, possibly by reorienting crystals or by creating new centers of nucleation, so that excessive grain growth does not occur during subsequent solution-heat-treatment.

In so far as known, the process of the invention may be successfully applied to articles formed of any heat-treatable magnesium-base alloy which tends to undergo germination on prolonged heating. In this connection, however, it may be noted that the tendency toward uncontrolled crystal growth is most common with cast metal, especially metal which has been locally strained by drastic chilling in the mold. The practice of superheating magnesium alloys in the molten state to effect grain refinement prior to casting also seriously aggravates, and may even

initiate, germination during subsequent heat-treatment of the casting. Commercial magnesium alloys containing from 8 to 14 per cent of aluminum as the major alloying element, especially those in which the usual 0.1 to 0.2 per cent manganese is absent, and to a lesser extent those alloys containing up to 4 per cent of zinc, as well as aluminum and the usual amount of manganese, appear to be particularly susceptible to sporadic grain growth. For this reason, the pre-treatment according to the invention is most commonly used as a preliminary step in the solution-heat-treatment of castings poured from superheated magnesium-aluminum-zinc alloys of the type mentioned.

Among the commercial magnesium-base alloys to which the invention is most frequently applied are: Dowmetal C., containing from 8.3 to 9.7 per cent aluminum, 1.7 to 2.3 per cent zinc, and about 0.1 per cent manganese; Dowmetal G, containing from 9 to 11 per cent of aluminum, up to 0.3 per cent zinc, about 0.1 per cent manganese; and Dowmetal R, containing from 8.3 to 9.7 per cent aluminum, about 0.2 per cent manganese, and up to 1.0 per cent zinc, the balance of each alloy being magnesium.

In practicing the invention, the casting or other article to be treated is first heated at a solution-heat-treating temperature, i. e. at a temperature well above the temperature limit of solid solubility of the subsisting concentration of the major alloying element in magnesium. In the case of magnesium-base alloys containing 8 to 14 per cent of aluminum, the preferred temperature is in the range of 715° to 800° F., being usually 750° to 770° F. The duration of this treatment should be sufficient to cause substantial solution of any second major phase present but not so long as to cause germination. With the magnesium-aluminum alloys mentioned, times of 0.2 hour to a maximum of about 8 hours are usually satisfactory, the longer times being required at the lower temperatures; 2 hours at 770° F. is a common procedure.

The preliminary heating is best accomplished in a standard furnace provided with a protective atmosphere, or in a molten salt bath. The metal should be raised to the required temperature as rapidly as possible, but, as in other heat-treatments of magnesium alloys, heating should not be so fast that the eutectic phase melts and "burns" before it goes into solid solution. For example, a heating time of about 2 hours may be necessary to raise a magnesium-aluminum alloy

casting from about 640° F. to a treatment temperature of 770° F.

After the brief partial solution-heat-treatment just described, the magnesium alloy article is cooled rapidly to an aging temperature or below and is then given an aging treatment for a time sufficient to effect substantial precipitation of a second phase. Cooling is ordinarily done in still air, although forced-draft or other means may be used. Aging may be carried out in conventional manner, i. e. by heating at a temperature below the temperature limit of solid solubility in magnesium of the existing concentration of the major alloying element. With magnesium alloys containing 8 to 14 per cent of aluminum, temperatures of 350° to 700° F. and times of 2 to 20 hours are effective, the higher temperatures requiring the shorter times.

Following the pre-heating and the aging steps, the castings or other articles may be given a conventional solution-heat-treatment, e. g. at 715° to 800° F. for 10 to 25 hours for magnesium-aluminum alloys, without undergoing substantial germination, a result usually not otherwise possible with alloys having germinative tendencies. The pretreatment according to the invention in general decreases somewhat the time required to effect the conventional solution-heat-treatment.

In particularly difficult cases of germination, as with castings subjected to extreme local chilling, it may occasionally be necessary to repeat the partial solution-heat-treating and aging steps of the invention one or more times in order entirely to prevent germination during prolonged solution-heat-treatment.

Regarding the invention from another viewpoint, it may be seen that the prevention of germination is accomplished essentially by interrupting an ordinary solution-heat-treatment prior to the occurrence of germination and subjecting the article to an aging temperature for a time sufficient to effect substantial precipitation-hardening before resuming the solution-heat-treatment.

The following example will further illustrate the invention but is not to be construed as limiting its scope:

#### Example

A considerable number of identical aircraft castings of intricate design were poured from a magnesium-base alloy containing 9.0 per cent aluminum and 2.0 per cent zinc which had been superheated at 1650° F. to effect grain refinement. After solution-heat-treatment at 770° F. for 18 hours, 70 per cent of the castings were found on inspection to have undergone serious germination.

In contrast, with an otherwise identical series of castings which were pre-heated at 770° F. for 2 hours and aged at 650° F. for 4 hours in accordance with the invention, and were then solution-heat-treated at 770° F. for 18 hours, less than 5 per cent of the castings showed even traces of germination.

It is to be understood that the foregoing description is illustrative rather than strictly limita-

tive, and that the invention is co-extensive in scope with the following claims.

What is claimed is:

1. An improved procedure for producing in an ungerminated condition solution-heat-treated articles formed of a heat-treatable magnesium-base alloy characterized by a tendency to undergo germination on prolonged heating, which comprises pre-heating the article at a solution-heat-treating temperature for a period sufficient to effect partial solution of a major second phase in the alloy but insufficient to produce appreciable germination, then subjecting it to an aging temperature for a time sufficient to effect substantial precipitation, and thereafter subjecting the article to solution-heat-treatment.
2. An improved procedure for producing in an ungerminated condition after solution-heat-treatment castings poured from a superheated heat-treatable magnesium-base alloy containing from 8 to 14 per cent aluminum and up to 4 per cent zinc as the major alloying elements, which comprises pre-heating the casting at a solution-heat-treating temperature of at least 715° F. for a period sufficient to effect partial solution of any second phase in the alloy but not exceeding about 8 hours, then cooling the casting rapidly and subjecting it to an aging temperature in the range 325° to 700° F. for a time sufficient to effect substantial precipitation, and thereafter subjecting the casting to solution-heat-treatment at a temperature of at least 715° F.
3. A process according to claim 2 in which the magnesium-base alloy contains from 8.3 to 9.7 per cent aluminum and from 1.7 to 2.3 per cent zinc.
4. A process according to claim 2 in which the magnesium-base alloy contains from 9 to 11 per cent aluminum and up to 0.3 per cent zinc.
5. A process according to claim 2 in which the magnesium-base alloy contains from 8.3 to 9.7 per cent aluminum and up to 1.0 per cent zinc.
6. In a process of solution-heat-treating castings formed of a heat-treatable magnesium-base alloy characterized by a tendency to undergo germination on prolonged heating, a pre-treatment for minimizing germination during subsequent heat-treatment which comprises heating the casting at a solution-heat-treating temperature for a time sufficient to effect partial solution of any second phase in the alloy but insufficient to cause appreciable germination, and then cooling the casting and subjecting it to an aging temperature for a time sufficient to effect substantial precipitation.
7. An improvement in the solution-heat-treatment of articles formed of a heat-treatable magnesium-base alloy characterized by a tendency to undergo germination on prolonged heating which comprises interrupting the solution-heat-treatment prior to the occurrence of appreciable germination and subjecting the article to an aging temperature for a time sufficient to effect substantial precipitation before resuming the solution-heat-treatment.

ROBERT S. BUSK.